

Jan. 23, 1945.

H. KALISING ET AL

2,367,871

GLASS ENVELOPE FOR ELECTRIC SUNLAMPS

Filed March 16, 1942

Fig. 1.



Fig. 2.



Inventors:

Harry Kalsing,

Hermann Krefft,

Kurt Larche,

by *John H. Anderson*  
Their Attorney.

## UNITED STATES PATENT OFFICE

2,367,871

GLASS ENVELOPE FOR ELECTRIC  
SUN LAMPS

Harry Kalsing, Weisswasser, Hermann Kreft,  
Berlin-Schöneberg, and Kurt Larché, Berlin-  
Tempelhof, Germany, assignors to General  
Electric Company, a corporation of New York

Application March 16, 1942, Serial No. 434,978  
In Germany December 22, 1939

2 Claims. (Cl. 106—53)

Our invention relates to sunlamps especially rich in ultraviolet radiation and more particularly to the glass envelopes of that type of ultraviolet electric sunlamp which is designed generally for nonprofessional use such as for general body exposure to improve the general health or for cosmetic purposes.

In lamps of the aforesaid type it is highly desirable to employ a glass envelope which will absorb as much as possible the bodily harmful strong radiations of the shorter wavelengths of the ultraviolet spectrum, generally those shorter than 280 mu, and yet transmit with as little energy loss as possible the medium and longer wavelengths. These shorter wavelength radiations have generally harmful effects which are difficult to guard against in the absence of professional supervision.

Although glasses possessing such transmission characteristics are known, most of them undergo some change in their spectral transmission characteristics during the operating life of the lamp while in some the change is very great. The result is that the same lamp may cause quite different biologic effects at different times during its operating life. Under such circumstances the user can rely neither upon the tables of exposure furnished with the lamp nor upon his experience with previous exposures. Neither can he rely upon the sensation during exposure as an indication of radiation intensity since the ultraviolet radiation generally becomes noticeable only after several hours.

These undesirable aging phenomena may be suppressed by the addition of small amounts of nickel oxide to a bulb of alkali-silicate glass in the manner described in United States Patent No. 2,212,879 issued August 27, 1940, to Harry Kalsing et al. By the present invention, however, we have not only obtained this desired result but also a spectral transmission characteristic curve of much more favorable shape.

It is therefore an object of our invention not only to avoid the uncertainty caused by the changing spectral character of the radiation from ultraviolet sunlamps by maintaining the spectral analysis of the lamp radiation constant during the entire life of the lamp but also to obtain, at the same time, a particularly advantageous transmission characteristic. This object is accomplished according to our invention by employing a bulb of alkali-silicate glass which contains from 5% to 20% of lead oxide along with a silica content of more than 60%. Further objects and ad-

vantages of our invention will appear from the following detailed description.

In the drawing, Fig. 1 shows a sunlamp of a type commonly in use constructed in accordance with our invention while Fig. 2 shows a typical spectral transmission curve of a glass made in accordance with our invention.

Referring more particularly to Fig. 1, the enveloping bulb 2, provided with a conventional threaded base 1 similar to that of an incandescent lamp, contains a spherical high pressure mercury lamp 3 and a coiled incandescent filament 4, which serves as a series resistance for limiting the discharge current. Lamp 3 is preferably constructed of a high melting point, ultraviolet transmitting glass, especially quartz glass, and has an inside diameter of about 8 millimeters. As in the usual lamp of this type, the lamp 3 contains fixed incandescent electrodes 5—5, which are preferably hollow tungsten bodies containing active oxides or other electron emitting substances, and, in addition to the usual filling of ignition gas, a drop of mercury 6. The size of the mercury drop is so chosen that during operation of the lamp an unsaturated vapor pressure of about 100 atmospheres is developed whereby the arc voltage rises to about 130 to 140 volts. The high pressure tube will then consume about 65 to 70 watts with a specific wall loading of its inner surface of more than 30 watts per square centimeter. The sunlamp may be connected to any convenient source of power with a voltage of the order of 220 or more and may have a power consumption of about 110 watts with an operating current of about 0.5 ampere. The series resistor 4 is preferably designed as an incandescent filament and not only serves to limit the discharge current but also furnishes additional radiation, especially heat radiation. Alternatively, the lamp 3 may be of the type disclosed in the United States Patent No. 2,094,694 to Cornelis Bol et al. or any of the high pressure mercury vapor type designed to operate at pressures from 1 to 50 atmospheres or more.

The enclosing bulb 2 may contain a gas filling as is customary with incandescent lamps and consists of an ultraviolet transmitting glass of the following constitution in accordance with our invention:

50 65 to 75%, preferably 72%  $\text{SiO}_2$   
10 to 15%, preferably 11.5%  $\text{K}_2\text{O}$   
4 to 8%, preferably 6%  $\text{Na}_2\text{O}$   
0 to 5%, preferably 0.5%  $\text{Al}_2\text{O}_3$   
55 5 to 15%, preferably 10%  $\text{PbO}$

The alkali content of the glass of more than 12% facilitates in a familiar manner the melting and also the working of the glass.

Where a small design of enclosing bulb 2 is desirable, it may be necessary to take into consideration a high temperature rise during the lamp operation. In that case, a lead oxide hard glass of the following composition may be used advantageously:

|                                      | Per cent |
|--------------------------------------|----------|
| SiO <sub>2</sub> -----               | 69.0     |
| B <sub>2</sub> O <sub>3</sub> -----  | 17.0     |
| Al <sub>2</sub> O <sub>3</sub> ----- | 1.2      |
| Sb <sub>2</sub> O <sub>3</sub> ----- | 1.1      |
| Na <sub>2</sub> O -----              | 1.7      |
| K <sub>2</sub> O -----               | 4.0      |
| PbO -----                            | 5.7      |
| As <sub>2</sub> O <sub>3</sub> ----- | 0.3      |
|                                      | 100.0    |

The transmission characteristics of enclosing bulbs of these compositions are very favorable. The spectral transmission curve is substantially flatter than those of glasses heretofore known and extends considerably into the short wave region before substantially complete cut-off obtains at about 250 mu. With the customary bulb wall thicknesses of about 0.5 to 1.0 millimeters, the absorption of wave lengths below 280 mu is practically complete. For example, with a bulb wall thickness of 0.7 mm. and a glass of the first-mentioned composition at the preferred proportions, we obtain the particularly sharp cut-off characteristic curve shown in Fig. 2 wherein relative energy transmission efficiencies are plotted as a function of wavelength.

As indicated by the curve itself, radiation below the wavelength 280 mu (millimicrons) is substantially absorbed and rendered harmless to the body, while at only slightly higher wavelengths of about 310 mu the transmission has reached a value of 80% of the total. This is particularly advantageous since it is the ultraviolet radiations above this approximate cut off range which are desirable for the purposes of sunlamps.

Sunlamps of the type shown can be used in the

usual sockets of incandescent lamps without external series resistance and can be used by laymen for home exposure without danger. They have, in addition, the advantage that the quality of the spectral radiation remains constant throughout the operating life.

For improving the color tone of the lamp radiation or the appearance of the lamp or for more or less strongly absorbing the visible radiation, 10 coloring matters may be added in the manner well known in the art. For example, cobalt oxide, nickel oxide or manganese oxide may be used. If a small amount of antimony monoxide or bismuth oxide is added to the bulb glass, these will function as substitutes for the lead oxide. Small amounts of these ingredients will permit a relatively large reduction of the lead oxide content. Of course, the bulb glass must be sufficiently free of such materials or impurities as iron oxide 15 which diminish the transmission of ultraviolet radiation.

It will be understood that the herein described glass may be used to advantage with many types of sunlamps; that the particular lamp herein described is illustrative of but one embodiment of our invention and is not to be construed as a limitation upon the scope of the appended claims.

What we claim as new and desire to secure by Letters Patent of the United States is:

1. An ultraviolet transmitting glass, impervious to ultraviolet radiations of wavelengths shorter than about 280 mu and having a substantially constant ultraviolet transmission characteristic, containing 72% SiO<sub>2</sub>, 11.5% K<sub>2</sub>O, 6% Na<sub>2</sub>O, 0.5% Al<sub>2</sub>O<sub>3</sub>, and 10% PbO.
2. An ultraviolet transmitting glass, impervious to ultraviolet radiations of wavelengths shorter than about 280 mu and having a substantially constant ultraviolet transmission characteristic, containing 69.0% SiO<sub>2</sub>, 17.0% B<sub>2</sub>O<sub>3</sub>, 1.2% Al<sub>2</sub>O<sub>3</sub>, 1.1% Sb<sub>2</sub>O<sub>3</sub>, 1.7% Na<sub>2</sub>O, 4.0% K<sub>2</sub>O, 5.7% PbO and 0.3% As<sub>2</sub>O<sub>3</sub>.

HARRY KALSING.  
HERMANN KREFFT.  
KURT LARCHE.